

## UNITED STATES PATENT OFFICE.

EDWIN C. WALLACE, OF WEST ROXBURY, MASSACHUSETTS.

## MANUFACTURE OF FUEL.

No Drawing.

Application filed June 10, 1920. Serial No. 387,930.

To all whom it may concern:

Be it known that I, EDWIN C. WALLACE, citizen of the United States, residing at West Roxbury, in the county of Suffolk and State 5 of Massachusetts, have invented certain new and useful Improvements in Manufacture of Fuel, of which the following is a specification.

The present invention relates to the production of briquet fuel, employing peat or similar somewhat wet material as one of the ingredients, a cementitious material, of the nature of Portland cement as another ingredient, and either finely-divided coal (e. 15 g., coal dust), partly dried peat, or other pulverulent or comminuted combustible material, as a third ingredient, the product being made up into the form of briquets of any desired size and shape. In this 20 specification where reference is made to the formation of briquets, this does not imply, or is not intended to imply, any particular size or shape. The briquets may be, and preferably are made into a size approximating that of coal ready for use in stoves or 25 furnaces, but if desired the briquets can, of course, be made considerably larger, and subsequently be crushed or broken. Such 30 practice, however, is generally not to be recommended, it being considered preferable to make the briquets directly into the size and shape in which they are to be finally used as fuel.

Ordinary wet peat as taken from the 35 bogs, contains a large amount of water. The amount of water varies greatly, different materials carrying from 75% to 90%, or even a slightly higher percentage than this, of water. After drying in air at ordinary 40 temperature for a considerable time, the peat will usually contain from 40 to 62% of water, and this water content is likewise variable, depending upon the particular kind of peat and the conditions of the 45 drying operation.

In drying peat down to what may be termed the "air dry" condition, there are certain chemical changes which take place whereby the material if added to water will 50 not reconstitute the original material, some of the properties having been changed, per-

haps by bacterial action or by oxidation produced in various ways.

In the preferred mode of carrying out the process of the present application, peat which has been partly dried in air so that the moisture content is reduced to approximately 40% is combined with peat containing a larger percentage of moisture and a previously prepared mixture of finely divided dry combustible matter, such as coal dust, and a cementing agent, such as Portland cement, capable of combining with and hardening in the presence of moisture.

While the proportions may vary within wide limits the mixed mass should be plastic so as to be readily molded.

It has been found that a mixture of 400 parts of peat (combined wet and partially dried) containing about 55% of moisture, 70 with 75 parts of a previously-prepared mixture of 90% bituminous coal (finely divided) and 10% of Portland cement, gives excellent results. By substituting about 20% of fine ground sawdust for coal in the 75 above mixture (i. e. a mixture of 70% coal, 20% sawdust, 10% Portland cement) the proportion of dry combustible material required was reduced to 50 parts thereof to 400 parts of the moist peat.

This mixture is then made up into balls, briquets, or the like, preferably using some pressure in molding the same (although high pressure is not necessary), after which the blocks or briquets are allowed to dry in 85 the open air. This drying may, under ordinary weather conditions require a week or longer. Tests made with the fuel prepared as described hereinbefore have shown it to compare favorably with ordinary coal. In 90 the molding operation, no very great pressure is necessary. In an experimental way it has been molded by hand, i. e., by squeezing a handful of the material at a time, in the manner of making ordinary snow-balls. 95

In place of the bituminous coal, there may be substituted sawdust, etc., other kinds of substantially dry carbonaceous matter, e. g., hard coal slack, culm, well dried peat, saw-dust, comminuted paper, paper pulp, 100 dry lignite, wood meal, chaff, straw, and the like, or mixtures of such materials, all in

a well dried condition. It is, however, preferable to use, with the substances just mentioned, a substantial content of dry, finely-divided coal. This mixture of the wet peat 5 with whatever dry material or materials are to be used (e. g., the 475 parts above mentioned) should be in the form of a plastic mass, of stiff putty-like, or stiff dough-like consistency.

10 The above mode of procedure, that is mixing partially dry peat with wet peat to produce a peat mixture of about 50 to 55% of water, which then, in turn is to be mixed with the mixture of dry combustible material and a cementing agent, is preferable to merely drying the entire body of peat down to 55% of water, since better control 15 of moisture content is obtainable and a far better final product is produced, which will dry much more quickly.

15 The Portland cement, this should be preferably mixed with the dry combustible matter and this mixture added to and mixed with the mixture of wet and dry peat. Portland 20 cement is here mentioned as an example of a suitable dry material, although other hydraulic dry plasters or cements may be employed, such as plaster of Paris, hydraulic lime, or in some cases even ordinary quick lime.

25 In making up the plastic mass, the Portland cement, or equivalent dry material, is first mixed, e. g., by grinding, with a dry combustible material, as above stated. This latter, during the final mixing operation, acts as an extending material for the cement (thus causing it to be much more thoroughly disseminated throughout the mass of wet peat). The dry cement accordingly will 30 gradually absorb from the wet peat, enough water to make the cement harden or set properly, however before the final setting of the cement, the mass is molded or shaped into briquets, balls or the like.

45 In the claims which follow hereinafter, by the term, "hydraulic", as applied to the cement and to the cementitious binder therein named, it is intended to describe or specify a cementitious substance which, when treated with water, tends to harden or set, and to distinguish such cementitious material from mucilaginous or sticky adhesives of the nature of the "glutin" described in 50 United States Patent No. 948812 and of the "pentosane" mentioned in United States Patent No. 773992. It is to be observed that the finely-divided coal serves not only to increase the calorific value of the fuel 55 hereinbefore described, but also to extend, distribute and disseminate the hydraulic cement throughout the mass of the mixture and to bring the hydraulic cement into intimate contact with the wet peat, from 60 which, when the cement-carrying coal is

intimately incorporated therewith, the hydraulic cement takes up the water necessary to cause it to harden and set and, in doing this, to bind the ingredients of the fuel into a hard, solid mass.

70

I claim—

1. A process which comprises mixing about 400 parts of peat having about 50% of water with about 75 parts of a mixture consisting of 90 parts of substantially dry combustible matter and 10 parts of dry hydraulic cement disseminated therethrough, forming into briquets and drying.

75

2. In the manufacture of briquet fuel, the improvement which comprises mixing a partially dried peat containing about 50 to 65% of water with a mixture consisting of substantially dry combustible matter and a dry, hydraulic cementitious binder disseminated therethrough, in such proportions as to produce with the peat a plastic mass, shaping the plastic mass and drying the product.

80

3. In the manufacture of briquet fuel, the improvement which comprises mixing peat containing between 40 and 65% of water, the peat comprising a mixture of a relatively wet peat and a relatively dry peat, with a less bulk of a mixture of a substantially dry combustible material and a dry, hydraulic cementitious binder disseminated therethrough, in such proportions as to produce with the peat a plastic mass, shaping the plastic mass and drying the product.

85

4. A process of making briquet fuel from material including somewhat wet vegetable material of the nature of peat, which comprises mixing with the wet material, a minor fraction only of its weight of a mixture containing relatively dry combustible matter and a dry calcareous cement capable of uniting with water to harden, such proportions being sufficient to produce a stiff dough-like mass, and forming the same into briquets, and thereafter allowing such briquets to dry.

90

5. A process of making fuel briquets from peat which comprises drying one portion of the peat, to substantially below 60% of water, mixing the same with another portion of the peat containing a substantially greater percentage of water than said first-mentioned portion, and with a dry pulverulent cementitious material which is capable of combining with water and hardening, incorporated with a dry extending material; such materials being mixed in such proportions as to produce a plastic mass, molding such mass into briquets and allowing such briquets to dry.

105

6. A process of making fuel briquets consisting largely of the dry matter of peat, which comprises mixing wet peat with peat which has been exposed to air and from

110

115

120

125

130

which a considerable proportion of the water has been dried out, such two materials being mixed in such relative proportions as to produce a mixture containing between 40% and 62% of water; separately mixing a calcareous cementitious binder with several times its weight of substantially dry combustible material; intimately mixing a large quantity of such first mentioned mixture with a small quantity of such second mixture, shaping the resulting plastic mass,

whereby the cementitious binder can absorb and combine with a part of the water of the peat, and drying the product at a low temperature.

In testimony whereof I hereunto affix my signature in the presence of two witnesses.

EDWIN C. WALLACE. [L.S.]

Witnesses:

E. W. DALEY,  
JOHN DEARBORN.